



US009970242B2

(12) **United States Patent**  
Narikawa et al.

(10) **Patent No.:** US 9,970,242 B2  
(45) **Date of Patent:** May 15, 2018

(54) **GALLING RESISTANT DRILL PIPE TOOL JOINT AND CORRESPONDING DRILL PIPE**

(71) **Applicant:** TENARIS CONNECTIONS B.V.,  
Amsterdam (NL)

(72) **Inventors:** Tomoyuki Narikawa, Kawasaki (JP);  
Tatsuo Ono, Kawasaki (JP); Koji  
Sakura, Kawasaki (JP); Toshihiko  
Fukui, Kawasaki (JP); Motohisa  
Yoshida, Kawasaki (JP); Takeshi  
Kuwano, Kawasaki (JP); Nobuo  
Kobayashi, Kawasaki (JP); Nobuhide  
Sato, Kawasaki (JP)

(73) **Assignee:** Tenaris Connections B.V., Amsterdam  
(NL)

(\*) **Notice:** Subject to any disclaimer, the term of this  
patent is extended or adjusted under 35  
U.S.C. 154(b) by 0 days. days.

(21) **Appl. No.:** 14/760,300

(22) **PCT Filed:** Jan. 11, 2013

(86) **PCT No.:** PCT/IB2013/050265

§ 371 (c)(1),

(2) Date: Jul. 10, 2015

(87) **PCT Pub. No.:** WO2014/108756

PCT Pub. Date: Jul. 17, 2014

(65) **Prior Publication Data**

US 2015/0368986 A1 Dec. 24, 2015

(51) **Int. Cl.**

E21B 17/042 (2006.01)

E21B 17/00 (2006.01)

(Continued)

(52) **U.S. Cl.**

CPC ..... E21B 17/042 (2013.01); E21B 17/00  
(2013.01); E21B 19/16 (2013.01); C25D 7/04  
(2013.01)

(58) **Field of Classification Search**

USPC ..... 166/380, 242.1; 285/333  
See application file for complete search history.

(56) **References Cited**

U.S. PATENT DOCUMENTS

141,451 A \* 8/1873 Speller ..... A22C 11/02  
452/42  
1,590,357 A 6/1926 Feisthamel  
(Continued)

FOREIGN PATENT DOCUMENTS

AR 0050159 A1 10/2006  
AT 388791 B 8/1989  
(Continued)

OTHER PUBLICATIONS

Fritz T et al, "Characterization of electroplated nickel",  
Microsystem Technologies, Dec. 31, 2002, vol. 9, No. 1-2, pp.  
87-91, Berlin, DE.

(Continued)

*Primary Examiner* — Taras P Bemko

(74) **Attorney, Agent, or Firm:** Knobbe Martens Olson  
& Bear LLP

(57) **ABSTRACT**

Disclosed herein are embodiments of a drill pipe tool joint and a drill pipe which are optimized for repeated make-up/break-out operations without the use of screw grease. Embodiments of the disclosure are environment friendly as well as having improved operating efficiency. In particular, the box and pin can be formed from different materials having different hardness.

**30 Claims, 5 Drawing Sheets**

HARDNESS RATIO AND NUMBER OF TIMES  
OF MAKE-UP AND BREAK-OUT



|      |                              |           |                   |              |         |                     |                              |
|------|------------------------------|-----------|-------------------|--------------|---------|---------------------|------------------------------|
| (51) | <b>Int. Cl.</b>              |           |                   |              |         |                     |                              |
|      | <b>E21B 19/16</b>            | (2006.01) |                   | 4,491,725 A  | 1/1985  | Pritchard           |                              |
|      | <b>C25D 7/04</b>             | (2006.01) |                   | 4,506,432 A  | 3/1985  | Smith               |                              |
|      |                              |           |                   | 4,526,628 A  | 7/1985  | Ohno et al.         |                              |
|      |                              |           |                   | 4,527,815 A  | 7/1985  | Frick               |                              |
|      |                              |           |                   | 4,564,392 A  | 1/1986  | Ohhashi et al.      |                              |
| (56) | <b>References Cited</b>      |           |                   | 4,570,982 A  | 2/1986  | Blose et al.        |                              |
|      | <b>U.S. PATENT DOCUMENTS</b> |           |                   | 4,591,195 A  | 5/1986  | Chelette et al.     |                              |
|      |                              |           |                   | 4,592,558 A  | 6/1986  | Hopkins             |                              |
|      |                              |           |                   | 4,601,491 A  | 7/1986  | Bell, Jr. et al.    |                              |
|      |                              |           |                   | 4,602,807 A  | 7/1986  | Bowers              |                              |
|      | 1,671,458 A                  | 5/1928    | Wilson            | 4,623,173 A  | 11/1986 | Handa et al.        |                              |
|      | 1,799,762 A                  | 1/1929    | Rathbun           | 4,629,218 A  | 12/1986 | Dubois              |                              |
|      | 1,999,706 A                  | 4/1935    | Spang             | 4,662,659 A  | 5/1987  | Blose et al.        |                              |
|      | 2,075,427 A                  | 3/1937    | Church            | 4,674,756 A  | 6/1987  | Fallon et al.       |                              |
|      | 2,211,173 A                  | 8/1940    | Shaffer           | 4,688,832 A  | 8/1987  | Ortloff et al.      |                              |
|      | 2,636,753 A                  | 4/1948    | Griffin           | 4,706,997 A  | 11/1987 | Carstensen          |                              |
|      | 2,487,241 A                  | 11/1949   | Hilton            | 4,710,245 A  | 12/1987 | Roether             |                              |
|      | 2,539,057 A                  | 1/1951    | Brown             | 4,721,536 A  | 1/1988  | Koch et al.         |                              |
|      | 2,567,113 A                  | 9/1951    | Kristensen        | 4,758,025 A  | 7/1988  | Frick               |                              |
|      | 2,631,871 A                  | 3/1953    | Stone             | 4,762,344 A  | 8/1988  | Perkins et al.      |                              |
|      | 2,634,943 A                  | 4/1953    | Gulick            | 4,812,182 A  | 3/1989  | Fang et al.         |                              |
|      | 2,841,429 A                  | 10/1955   | McCuistion        | 4,814,141 A  | 3/1989  | Imai et al.         |                              |
|      | 2,766,998 A                  | 10/1956   | Watts et al.      | 4,844,517 A  | 7/1989  | Beiley et al.       |                              |
|      | 2,916,306 A                  | 12/1959   | Rickard           | 4,856,828 A  | 8/1989  | Kessler et al.      |                              |
|      | 2,992,021 A                  | 7/1961    | Nay               | 4,955,645 A  | 9/1990  | Weems               |                              |
|      | 2,992,613 A                  | 7/1961    | Bodine            | 4,958,862 A  | 9/1990  | Cappelli et al.     |                              |
|      | 3,016,250 A                  | 1/1962    | Franck            | 4,988,127 A  | 1/1991  | Cartensen           |                              |
|      | 3,041,088 A                  | 6/1962    | Brandon           | 5,007,665 A  | 4/1991  | Bovisio et al.      |                              |
|      | 3,054,628 A                  | 9/1962    | Hardy et al.      | 5,067,874 A  | 11/1991 | Foote               |                              |
|      | 3,150,889 A                  | 9/1964    | Watts             | 5,137,310 A  | 8/1992  | Noel et al.         |                              |
|      | 3,219,354 A                  | 11/1965   | Kazienko          | 5,143,381 A  | 9/1992  | Temple              |                              |
|      | 3,266,824 A                  | 8/1966    | Nealy             | 5,154,534 A  | 10/1992 | Guerin et al.       |                              |
|      | 3,307,860 A                  | 3/1967    | Blount et al.     | 5,180,008 A  | 1/1993  | Aldridge et al.     |                              |
|      | 3,316,395 A                  | 4/1967    | Lavin             | 5,191,911 A  | 3/1993  | Dubois              |                              |
|      | 3,316,396 A                  | 4/1967    | Lavin             | 5,242,199 A  | 9/1993  | Hann et al.         |                              |
|      | 3,325,174 A                  | 6/1967    | Weaver            | 5,328,158 A  | 7/1994  | Lewis et al.        |                              |
|      | 3,362,731 A                  | 1/1968    | Gasche et al.     | 5,348,350 A  | 9/1994  | Blose et al.        |                              |
|      | 3,366,392 A                  | 1/1968    | Kennel            | 5,352,406 A  | 10/1994 | Barteri et al.      |                              |
|      | 3,413,166 A                  | 11/1968   | Zackay et al.     | 5,360,239 A  | *       | 11/1994             | Klementich ..... F16L 15/001 |
|      | 3,489,437 A                  | 1/1970    | Duret             |              |         | 285/328             |                              |
|      | 3,512,789 A                  | 5/1970    | Tanner            | 5,445,683 A  | *       | 8/1995              | Tahara ..... C23C 8/24       |
|      | 3,552,781 A                  | 1/1971    | Helland           |              |         | 148/317             |                              |
|      | 3,572,777 A                  | 3/1971    | Blose et al.      |              |         |                     |                              |
|      | 3,575,430 A                  | 4/1971    | Alpine            | 5,454,883 A  | 10/1995 | Yoshie et al.       |                              |
|      | 3,592,491 A                  | 7/1971    | Glover            | 5,505,502 A  | 4/1996  | Smith et al.        |                              |
|      | 3,599,931 A                  | 8/1971    | Hanson            | 5,515,707 A  | 5/1996  | Smith               |                              |
|      | 3,655,465 A                  | 4/1972    | Snape et al.      | 5,538,566 A  | 7/1996  | Gallagher           |                              |
|      | 3,733,093 A                  | 5/1973    | Seiler            | 5,592,988 A  | 1/1997  | Meroni et al.       |                              |
|      | 3,810,793 A                  | 5/1974    | Heller            | 5,598,735 A  | 2/1997  | Saito et al.        |                              |
|      | 3,854,760 A                  | 12/1974   | Duret             | 5,653,452 A  | 8/1997  | Järvenkylä          |                              |
|      | 3,889,989 A                  | 6/1975    | Legris et al.     | 5,712,706 A  | 1/1998  | Castore et al.      |                              |
|      | 3,891,224 A                  | 6/1975    | Ditcher           | 5,794,985 A  | 8/1998  | Mallis              |                              |
|      | 3,893,919 A                  | 7/1975    | Flegel et al.     | 5,810,401 A  | 9/1998  | Mosing et al.       |                              |
|      | 3,915,697 A                  | 10/1975   | Giuliani et al.   | 5,860,680 A  | 1/1999  | Drijver et al.      |                              |
|      | 3,918,726 A                  | 11/1975   | Kramer            | 5,879,030 A  | 3/1999  | Clayson et al.      |                              |
|      | 3,986,731 A                  | 10/1976   | DeHoff            | 5,879,474 A  | 3/1999  | Bhadeshia et al.    |                              |
|      | 4,014,568 A                  | 3/1977    | Carter et al.     | 5,944,921 A  | 8/1999  | Cumino et al.       |                              |
|      | 4,147,368 A                  | 4/1979    | Baker et al.      | 5,993,570 A  | 11/1999 | Gray                |                              |
|      | 4,163,290 A                  | 7/1979    | Sutherlin et al.  | 6,006,789 A  | 12/1999 | Toyooka et al.      |                              |
|      | 4,219,204 A                  | 8/1980    | Pippert           | 6,030,470 A  | 2/2000  | Hensger et al.      |                              |
|      | 4,231,555 A                  | 11/1980   | Saito             | 6,044,539 A  | 4/2000  | Guzowsk             |                              |
|      | 4,299,412 A                  | 10/1981   | Parmann           | 6,045,165 A  | 4/2000  | Sugino et al.       |                              |
|      | 4,305,059 A                  | 12/1981   | Benton            | 6,056,324 A  | 5/2000  | Reimert et al.      |                              |
|      | 4,310,163 A                  | 1/1982    | Pippert           | 6,070,912 A  | 6/2000  | Latham              |                              |
|      | 4,336,081 A                  | 6/1982    | Hijikata et al.   | 6,173,968 B1 | 1/2001  | Nelson et al.       |                              |
|      | 4,345,739 A                  | 8/1982    | Wheatley          | 6,188,037 B1 | 2/2001  | Hamada et al.       |                              |
|      | 4,354,882 A                  | 10/1982   | Greer             | 6,196,530 B1 | 3/2001  | Muhr et al.         |                              |
|      | 4,366,971 A                  | 1/1983    | Lula              | 6,217,676 B1 | 4/2001  | Takabe et al.       |                              |
|      | 4,368,894 A                  | 1/1983    | Parmann           | 6,248,187 B1 | 6/2001  | Asahi et al.        |                              |
|      | 4,373,750 A                  | 2/1983    | Mantelle et al.   | 6,257,056 B1 | 7/2001  | Shibayama et al.    |                              |
|      | 4,376,528 A                  | 3/1983    | Ohshimatai et al. | 6,267,828 B1 | 7/2001  | Kushida et al.      |                              |
|      | 4,379,482 A                  | 4/1983    | Suzuki et al.     | 6,311,965 B1 | 11/2001 | Muhr et al.         |                              |
|      | 4,384,737 A                  | 5/1983    | Reusser           | 6,331,216 B1 | 12/2001 | Toyooka et al.      |                              |
|      | 4,406,561 A                  | 9/1983    | Ewing             | 6,347,814 B1 | 2/2002  | Cerruti             |                              |
|      | 4,407,681 A                  | 10/1983   | Ina et al.        | 6,349,979 B1 | 2/2002  | Noel et al.         |                              |
|      | 4,426,095 A                  | 1/1984    | Buttner           | 6,384,388 B1 | 5/2002  | Anderson et al.     |                              |
|      | 4,445,265 A                  | 5/1984    | Olson et al.      | 6,412,831 B1 | 7/2002  | Noel et al.         |                              |
|      | 4,468,309 A                  | 6/1984    | White             | 6,447,025 B1 | 9/2002  | Smith               |                              |
|      | 4,473,471 A                  | 9/1984    | Robichaud et al.  | 6,478,344 B2 | 11/2002 | Pallini, Jr. et al. |                              |
|      | 4,475,839 A                  | 10/1984   | Strandberg        | 6,481,760 B1 | 11/2002 | Noel et al.         |                              |

| (56)                  | References Cited            |                        |                 |                                  |              |  |  |
|-----------------------|-----------------------------|------------------------|-----------------|----------------------------------|--------------|--|--|
| U.S. PATENT DOCUMENTS |                             |                        |                 |                                  |              |  |  |
| 6,494,499 B1          | 12/2002 Galle, Sr. et al.   | 2002/0011284 A1        | 1/2002          | Von Hagen et al.                 |              |  |  |
| 6,514,359 B2          | 2/2003 Kawano               | 2002/0153671 A1        | 10/2002         | Raymond et al.                   |              |  |  |
| 6,527,056 B2          | 3/2003 Newman               | 2002/0158469 A1        | 10/2002         | Mannella et al.                  |              |  |  |
| 6,550,822 B2          | 4/2003 Mannella et al.      | 2003/0019549 A1        | 1/2003          | Turconi et al.                   |              |  |  |
| 6,557,906 B1          | 5/2003 Carcagno             | 2003/0111146 A1        | 6/2003          | Kusinski et al.                  |              |  |  |
| 6,558,484 B1 *        | 5/2003 Onoe .....           | C21D 9/0093<br>148/333 | 2003/0116238 A1 | 6/2003                           | Fujita       |  |  |
| 6,581,940 B2          | 6/2003 Dittel               | 2003/0155052 A1        | 8/2003          | Kondo et al.                     |              |  |  |
| 6,632,296 B2          | 10/2003 Yoshinaga et al.    | 2003/0165098 A1        | 9/2003          | Ohara et al.                     |              |  |  |
| 6,648,991 B2          | 11/2003 Turconi et al.      | 2003/0168859 A1        | 9/2003          | Watts                            |              |  |  |
| 6,669,285 B1          | 12/2003 Park et al.         | 2004/0118490 A1        | 6/2004          | Klueh et al.                     |              |  |  |
| 6,669,789 B1          | 12/2003 Edelman et al.      | 2004/0118569 A1        | 6/2004          | Brill et al.                     |              |  |  |
| 6,682,610 B1          | 1/2004 Inoue                | 2004/0131876 A1        | 7/2004          | Ohgami et al.                    |              |  |  |
| 6,683,834 B2          | 1/2004 Ohara et al.         | 2004/0139780 A1        | 7/2004          | Cai et al.                       |              |  |  |
| 6,709,534 B2          | 3/2004 Kusinski et al.      | 2004/0151608 A1        | 8/2004          | Vogt et al.                      |              |  |  |
| 6,752,436 B1          | 6/2004 Verdillon            | 2004/0195835 A1        | 10/2004         | Noel et al.                      |              |  |  |
| 6,755,447 B2          | 6/2004 Galle, Jr. et al.    | 2004/0262919 A1        | 12/2004         | Dutilleul et al.                 |              |  |  |
| 6,764,108 B2          | 7/2004 Ernst et al.         | 2005/0012278 A1        | 1/2005          | Delange                          |              |  |  |
| 6,767,417 B2          | 7/2004 Fujita et al.        | 2005/0076975 A1        | 4/2005          | Lopez et al.                     |              |  |  |
| 6,814,358 B2          | 11/2004 Keck                | 2005/0087269 A1        | 4/2005          | Merwin                           |              |  |  |
| 6,851,727 B2          | 2/2005 Carcagno et al.      | 2005/0093250 A1        | 5/2005          | Santi et al.                     |              |  |  |
| 6,857,668 B2          | 2/2005 Otten et al.         | 2005/0166986 A1        | 8/2005          | Dell'erba et al.                 |              |  |  |
| 6,883,804 B2          | 4/2005 Cobb                 | 2006/0006600 A1        | 1/2006          | Roussie                          |              |  |  |
| 6,905,150 B2          | 6/2005 Carcagno et al.      | 2006/0124211 A1        | 6/2006          | Takano et al.                    |              |  |  |
| 6,921,110 B2          | 7/2005 Morotti et al.       | 2006/0137781 A1        | 6/2006          | Kusinski et al.                  |              |  |  |
| 6,958,099 B2          | 10/2005 Nakamura et al.     | 2006/0169368 A1        | 8/2006          | Lopez et al.                     |              |  |  |
| 6,971,681 B2          | 12/2005 Dell'erba et al.    | 2006/0231168 A1        | 10/2006         | Nakamura et al.                  |              |  |  |
| 6,991,267 B2          | 1/2006 Ernst et al.         | 2006/0243355 A1        | 11/2006         | Haiderer et al.                  |              |  |  |
| 7,014,223 B2          | 3/2006 Della Pina et al.    | 2006/0273586 A1        | 12/2006         | Reynolds, Jr. et al.             |              |  |  |
| 7,066,499 B2          | 6/2006 Della Pina et al.    | 2007/0039149 A1        | 2/2007          | Roussie                          |              |  |  |
| 7,074,283 B2          | 7/2006 Omura                | 2007/0089813 A1        | 4/2007          | Tivelli                          |              |  |  |
| 7,083,686 B2          | 8/2006 Itou                 | 2007/0137736 A1        | 6/2007          | Omura et al.                     |              |  |  |
| 7,108,063 B2          | 9/2006 Carstensen           | 2007/0200345 A1        | 8/2007          | Toscano et al.                   |              |  |  |
| 7,118,637 B2          | 10/2006 Kusinski et al.     | 2007/0216126 A1        | 9/2007          | Lopez et al.                     |              |  |  |
| 7,182,140 B2          | 2/2007 Wood                 | 2007/0246219 A1        | 10/2007         | Manella et al.                   |              |  |  |
| 7,214,278 B2          | 5/2007 Kusinski et al.      | 2008/0047635 A1        | 2/2008          | Konda et al.                     |              |  |  |
| 7,255,374 B2          | 8/2007 Carcagno et al.      | 2008/0115863 A1        | 5/2008          | McCrink et al.                   |              |  |  |
| 7,264,684 B2          | 9/2007 Numata et al.        | 2008/0129044 A1        | 6/2008          | Carcagno et al.                  |              |  |  |
| 7,284,770 B2          | 10/2007 Dell'erba et al.    | 2008/0219878 A1        | 9/2008          | Konda et al.                     |              |  |  |
| 7,310,867 B2          | 12/2007 Corbett, Jr.        | 2008/0226396 A1        | 9/2008          | Garcia et al.                    |              |  |  |
| 7,431,347 B2          | 10/2008 Ernst et al.        | 2008/0226491 A1        | 9/2008          | Satou et al.                     |              |  |  |
| 7,464,449 B2          | 12/2008 Santi et al.        | 2008/0264129 A1        | 10/2008         | Cheppe et al.                    |              |  |  |
| 7,475,476 B2          | 1/2009 Roussie              | 2008/0303274 A1        | 12/2008         | Mazzaferro et al.                |              |  |  |
| 7,478,842 B2          | 1/2009 Reynolds, Jr. et al. | 2008/0314481 A1        | 12/2008         | Garcia et al.                    |              |  |  |
| 7,506,900 B2          | 3/2009 Carcagno et al.      | 2009/0010794 A1        | 1/2009          | Turconi et al.                   |              |  |  |
| 7,621,034 B2          | 11/2009 Roussie             | 2009/0033087 A1 *      | 2/2009          | Carcagno et al. .... E21B 17/042 |              |  |  |
| 7,635,406 B2          | 12/2009 Numata et al.       |                        | 285/55          |                                  |              |  |  |
| 7,735,879 B2          | 6/2010 Toscano et al.       | 2009/0047166 A1        | 2/2009          | Tomomatsu et al.                 |              |  |  |
| 7,744,708 B2          | 6/2010 Lopez et al.         | 2009/0101242 A1        | 4/2009          | Lopez et al.                     |              |  |  |
| 7,752,416 B2          | 7/2010 Mazzaferro et al.    | 2010/0136363 A1        | 6/2010          | Valdez et al.                    |              |  |  |
| 7,753,416 B2          | 7/2010 Mazzaferro et al.    | 2010/0172717 A1 *      | 7/2010          | Corbett .....                    | F16B 29/00   |  |  |
| 7,862,667 B2          | 1/2011 Turconi et al.       |                        | 411/366.1       |                                  |              |  |  |
| 8,002,910 B2          | 8/2011 Tivelli et al.       | 2010/0181727 A1        | 7/2010          | Santi et al.                     |              |  |  |
| 8,007,601 B2          | 8/2011 Lopez et al.         | 2010/0181761 A1        | 7/2010          | Santi et al.                     |              |  |  |
| 8,007,603 B2          | 8/2011 Garcia et al.        | 2010/0187808 A1        | 7/2010          | Santi                            |              |  |  |
| 8,016,362 B2          | 9/2011 Itoga                | 2010/0193085 A1        | 8/2010          | Garcia                           |              |  |  |
| 8,215,680 B2          | 7/2012 Nestor               | 2010/0206553 A1        | 8/2010          | Bailey et al.                    |              |  |  |
| 8,262,094 B2          | 9/2012 Beele                | 2010/0294401 A1        | 11/2010         | Gomez                            |              |  |  |
| 8,262,140 B2          | 9/2012 Santi et al.         | 2010/0319814 A1        | 12/2010         | Perez                            |              |  |  |
| 8,317,946 B2          | 11/2012 Arai et al.         | 2010/0327550 A1        | 12/2010         | Lopez                            |              |  |  |
| 8,328,958 B2          | 12/2012 Turconi et al.      | 2011/0008101 A1        | 1/2011          | Santi et al.                     |              |  |  |
| 8,333,409 B2          | 12/2012 Santi et al.        | 2011/0041581 A1        | 2/2011          | Santi                            |              |  |  |
| 8,414,715 B2          | 4/2013 Altschuler et al.    | 2011/0042946 A1        | 2/2011          | Santi                            |              |  |  |
| 8,544,304 B2          | 10/2013 Nestor              | 2011/0077089 A1 *      | 3/2011          | Hirai .....                      | B60B 27/0005 |  |  |
| 8,636,856 B2          | 1/2014 Altschuler et al.    |                        | 464/139         |                                  |              |  |  |
| 8,821,653 B2          | 9/2014 Anelli et al.        | 2011/0097235 A1        | 4/2011          | Turconi et al.                   |              |  |  |
| 8,840,152 B2          | 9/2014 Carcagno et al.      | 2011/0133449 A1        | 6/2011          | Mazzaferro                       |              |  |  |
| 8,926,771 B2          | 1/2015 Agazzi               | 2011/0233925 A1        | 9/2011          | Pina                             |              |  |  |
| 9,004,544 B2          | 4/2015 Carcagno et al.      | 2011/0233926 A1        | 9/2011          | Carcagno                         |              |  |  |
| 9,163,296 B2          | 10/2015 Valdez et al.       | 2011/0247733 A1        | 10/2011         | Arai et al.                      |              |  |  |
| 9,187,811 B2          | 11/2015 Gomez et al.        | 2011/0259482 A1        | 10/2011         | Peters et al.                    |              |  |  |
| 9,188,252 B2          | 11/2015 Altschuler et al.   | 2011/0284137 A1        | 11/2011         | Kami et al.                      |              |  |  |
| 9,222,156 B2          | 12/2015 Altschuler et al.   | 2012/0032435 A1        | 2/2012          | Carcagno                         |              |  |  |
| 9,383,045 B2          | 7/2016 Santi et al.         | 2012/0199255 A1        | 8/2012          | Anelli                           |              |  |  |
| 2001/0035235 A1       | 11/2001 Kawano              | 2012/0204994 A1        | 8/2012          | Anelli                           |              |  |  |
|                       |                             | 2012/0211132 A1        | 8/2012          | Altschuler                       |              |  |  |
|                       |                             | 2013/0264123 A1        | 10/2013         | Altschuler                       |              |  |  |
|                       |                             | 2014/0021244 A1        | 1/2014          | DuBois                           |              |  |  |
|                       |                             | 2014/0027497 A1        | 1/2014          | Rowland et al.                   |              |  |  |
|                       |                             | 2014/0272448 A1        | 9/2014          | Valdez et al.                    |              |  |  |

| (56) | References Cited                                            | JP | 01 259125 A2   | 10/1989 |
|------|-------------------------------------------------------------|----|----------------|---------|
|      | U.S. PATENT DOCUMENTS                                       | JP | 01 283322 A2   | 11/1989 |
|      | 2014/0299235 A1 10/2014 Anelli                              | JP | 05-098350      | 12/1990 |
|      | 2014/0299236 A1 10/2014 Anelli                              | JP | 403006329 A    | 1/1991  |
|      | 2015/0061287 A1* 3/2015 Yoshikawa ..... E21B 17/042 285/334 | JP | 04 021718 A2   | 1/1992  |
|      | 2015/0368986 A1 12/2015 Narikawa                            | JP | 04 107214      | 4/1992  |
|      | 2016/0024625 A1 1/2016 Valdez                               | JP | 04 231414 A2   | 8/1992  |
|      | 2016/0102856 A1 4/2016 Minami                               | JP | 05 287381 A2   | 11/1993 |
|      |                                                             | JP | H06-042645     | 2/1994  |
|      |                                                             | JP | 06-093339      | 4/1994  |
|      |                                                             | JP | 06 172859 A2   | 6/1994  |
|      |                                                             | JP | 06-220536      | 8/1994  |
|      |                                                             | JP | 07 041856 A2   | 2/1995  |
|      |                                                             | JP | 07-139666      | 5/1995  |
|      |                                                             | JP | 07 197125 A2   | 8/1995  |
|      | FOREIGN PATENT DOCUMENTS                                    | JP | 08 311551      | 11/1996 |
| CA   | 2319926 7/2008                                              | JP | 09 067624 A2   | 3/1997  |
| CN   | 1401809 3/2003                                              | JP | 09-235617      | 9/1997  |
| CN   | 1487112 4/2004                                              | JP | 2704042        | 10/1997 |
| CN   | 101480671 7/2009                                            | JP | 10 140250      | 5/1998  |
| CN   | 101542002 9/2009                                            | JP | 10176239       | 6/1998  |
| CN   | 101613829 A 12/2009                                         | JP | 10 280037 A    | 10/1998 |
| CN   | 101413089 11/2010                                           | JP | 11 050148 A    | 2/1999  |
| DE   | 3310226 A1 10/1984                                          | JP | 11140580       | 5/1999  |
| DE   | 4446806 5/1996                                              | JP | 11229079       | 8/1999  |
| EA   | 010037 6/2008                                               | JP | 2000-063940    | 2/2000  |
| EA   | 012256 8/2009                                               | JP | 2000-178645    | 6/2000  |
| EP   | 0 032 265 7/1981                                            | JP | 2000-248337 A  | 9/2000  |
| EP   | 0 092 815 11/1983                                           | JP | 2000-313919 A2 | 11/2000 |
| EP   | 0 104 720 4/1984                                            | JP | 2001-131698    | 5/2001  |
| EP   | 0 159 385 10/1985                                           | JP | 2001-164338    | 6/2001  |
| EP   | 0 309 179 3/1989                                            | JP | 2001-172739 A2 | 6/2001  |
| EP   | 0 340 385 11/1989                                           | JP | 2001-271134    | 10/2001 |
| EP   | 0 329 990 11/1992                                           | JP | 2002-096105 A2 | 4/2002  |
| EP   | 0 658 632 6/1995                                            | JP | 2002-130554    | 5/2002  |
| EP   | 0 753 595 1/1997                                            | JP | 2003-074763    | 3/2003  |
| EP   | 0 788 850 8/1997                                            | JP | 2004-011009    | 1/2004  |
| EP   | 0 828 007 3/1998                                            | JP | 60 174822      | 9/2005  |
| EP   | 0 989 196 3/2000                                            | KR | 0245031        | 3/2000  |
| EP   | 1 008 660 6/2000                                            | KZ | 1418 B         | 12/1994 |
| EP   | 01 027 944 8/2000                                           | KZ | 2506 B         | 9/1995  |
| EP   | 1 065 423 1/2001                                            | KZ | 2673 B         | 12/1995 |
| EP   | 1 277 848 1/2003                                            | UA | 51138 A        | 11/2002 |
| EP   | 1 288 316 3/2003                                            | WO | WO 1984/002947 | 8/1984  |
| EP   | 1 296 088 3/2003                                            | WO | WO 1994/29627  | 12/1994 |
| EP   | 1 362977 11/2003                                            | WO | WO 1996/22396  | 7/1996  |
| EP   | 1 413 639 4/2004                                            | WO | WO 2000/06931  | 2/2000  |
| EP   | 1 705 415 9/2006                                            | WO | WO 2000/70107  | 11/2000 |
| EP   | 1 717 324 11/2006                                           | WO | WO 2001/075345 | 10/2001 |
| EP   | 1 726 861 11/2006                                           | WO | WO 2001/88210  | 11/2001 |
| EP   | 1 914 324 4/2008                                            | WO | WO 2002/29290  | 4/2002  |
| EP   | 1554518 B1 1/2009                                           | WO | WO 2002/035128 | 5/2002  |
| EP   | 2 028 284 2/2009                                            | WO | WO 2002/068854 | 9/2002  |
| EP   | 2 133 442 12/2009                                           | WO | WO 2002/086369 | 10/2002 |
| EP   | 2 216 576 A1 8/2010                                         | WO | WO 2002/093045 | 11/2002 |
| EP   | 2 239 343 10/2010                                           | WO | WO 2003/033856 | 4/2003  |
| EP   | 2325435 10/2012                                             | WO | WO 2003/048623 | 6/2003  |
| FR   | 1 149 513 A 12/1957                                         | WO | WO 2003/060198 | 7/2003  |
| FR   | 2 704 042 A 10/1994                                         | WO | WO 2003/087646 | 10/2003 |
| FR   | 2 848 282 A1 6/2004                                         | WO | WO 2004/023020 | 3/2004  |
| FR   | 2855587 12/2004                                             | WO | WO 2004/031420 | 4/2004  |
| GB   | 498 472 1/1939                                              | WO | WO 2004/033951 | 4/2004  |
| GB   | 1 398 214 6/1973                                            | WO | WO 2004/053376 | 6/2004  |
| GB   | 1 428 433 3/1976                                            | WO | WO 2004/097059 | 11/2004 |
| GB   | 2 104 919 A 3/1983                                          | WO | WO 2004/109173 | 12/2004 |
| GB   | 2 234 308 A 1/1991                                          | WO | WO 2005/098300 | 10/2005 |
| GB   | 2 276 647 10/1994                                           | WO | WO 2006/087361 | 4/2006  |
| GB   | 2 388 169 A 11/2003                                         | WO | WO 2006/078768 | 7/2006  |
| JP   | 58-187684 12/1983                                           | WO | WO 2007/002576 | 1/2007  |
| JP   | 60-086209 5/1985                                            | WO | WO 2007/017082 | 2/2007  |
| JP   | S 60 116796 A 6/1985                                        | WO | WO 2007/017161 | 2/2007  |
| JP   | 60-215719 A 10/1985                                         | WO | WO 2007/026970 | 3/2007  |
| JP   | 36025719 10/1985                                            | WO | WO 2007/028443 | 3/2007  |
| JP   | S61-103061 5/1986                                           | WO | WO 2007/034063 | 3/2007  |
| JP   | 61270355 11/1986                                            | WO | WO 2007/063079 | 6/2007  |
| JP   | 63004046 A2 1/1988                                          | WO | WO 2008/003000 | 1/2008  |
| JP   | 63004047 A2 1/1988                                          | WO | WO 2008/090411 | 7/2008  |
| JP   | 63230847 A2 9/1988                                          | WO | WO 2008/108263 | 9/2008  |
| JP   | 63230851 A2 9/1988                                          | WO | WO 2008/110494 | 9/2008  |
| JP   | 01 259124 A2 10/1989                                        | WO | WO 2008/110494 | 9/2008  |

(56)

## References Cited

## FOREIGN PATENT DOCUMENTS

|    |                |         |
|----|----------------|---------|
| WO | WO 2008/127084 | 10/2008 |
| WO | WO 2009/000851 | 12/2008 |
| WO | WO 2009/000766 | 1/2009  |
| WO | WO 2009/010507 | 1/2009  |
| WO | WO 2009/027308 | 3/2009  |
| WO | WO 2009/027309 | 3/2009  |
| WO | WO 2009/044297 | 4/2009  |
| WO | WO 2009/065432 | 5/2009  |
| WO | WO 2009/106623 | 9/2009  |
| WO | WO 2010/061882 | 6/2010  |
| WO | WO 2010/122431 | 10/2010 |
| WO | WO 2013/007729 | 1/2013  |

## OTHER PUBLICATIONS

- Kazutoshi Ohashi et al, "Evaluation of r-value of steels using Vickers hardness test", Journal of Physics: Conference Series, Aug. 7, 2012, p. 12045, vol. 379, No. 1, Institute of Physics Publishing, Bristol, GB.
- International Search Report for International Application No. PCT/IB2013/050265, dated Oct. 28, 2013.
- "Specifications for Threading, Gauging and Thread Inspection of Casing, Tubing, and Line Pipe Threads," American Petroleum Institute, Specification 5B, Apr. 2008, 15th Edition (Excerpts Only).
- Chang, L.C., "Microstructures and reaction kinetics of bainite transformation in Si-rich steels," XP0024874, Materials Science and Engineering, vol. 368, No. 1-2, Mar. 15, 2004, pp. 175-182, Abstract, Table 1.
- Extrait du Catalogue N 940, 1994.
- "Seamless Steel Tubes for Pressure Purposes—Technical Delivery Conditions—Part 1: Non-alloy Steel Tubes with Specified Room Temperature Properties" British Standard BS EN 10216-1:2002 E:1-26, published May 2002.
- "Seamless Steel Tubes for Pressure Purposes—Technical Delivery Conditions—Part 2: Non-alloy and Alloy Steel Tubes with Specified Elevated Temperature Properties" British Standard BS EN 10216-2:2002+A2:2007:E:1-45, published Aug. 2007.
- "Seamless Steel Tubes for Pressure Purposes—Technical Delivery Conditions—Part 3: Alloy Fine Grain Steel Tubes" British Standard BS EN 10216-3:2002 +A1:2004 E:1-34, published Mar. 2004.
- "Seamless Steel Tubes for Pressure Purposes—Technical Delivery Conditions—Part 4: Non-alloy and Alloy Steel Tubes with Specified Low Temperature Properties" British Standard BS EN 10216-4:2002 + A1:2004 E:1-30, published Mar. 2004.
- Aggarwal, R. K., et al.: "Qualification of Solutions for Improving Fatigue Life at SCR Touch Down Zone", Deep Offshore Technology Conference, Nov. 8-10, 2005, Vitoria, Espirito Santo, Brazil, in 12 pages.
- Anelli, E., D. Colleuori, M. Pontremoli, G. Cumino, A. Izquierdo, H. Quintanilla, "Metallurgical design of advanced heavy wall seamless pipes for deep-water applications", 4th International Conference on Pipeline Technology, May 9 to 13, 2004, Ostend, Belgium.
- Asahi, et al., Development of Ultra-high-strength Linepipe, X120, Nippon Steel Technical Report, Jul. 2004, Issue 90, pp. 82-87.
- ASM Handbook, Mechanical Tubing and Cold Finishing, Metals Handbook Desk Edition, (2000), 5 pages.
- ASTM A 213/A 213M "Standard Specification for Seamless Ferritic and Austenitic Alloy-Steel Boiler, Superheater, and Heat-Exchanger Tubes".
- ASTM A182/A182M "Standard Specification for Forged or Rolled Alloy and Stainless Steel Pipe Flanges, Forged Fittings, and Valves and Parts for High-Temperature Service".
- ASTM A336/A336M "Standard Specification for Alloy Steel Forgings for Pressure and High-Temperature Parts".
- ASTM A355 which is related to "Seamless Ferritic Alloy—Steel Pipe for High-Temperature Service".
- Bai, M., D. Liu, Y. Lou, X. Mao, L. Li, X. Huo, "Effects of Ti addition on low carbon hot strips produced by CSP process", Journal of University of Science and Technology Beijing, 2006, vol. 13, N° 3, p. 230.
- Beretta, Stefano et al., "Fatigue Assessment of Tubular Automotive Components in Presence of Inhomogeneities", Proceedings of IMECE2004, ASME International Mechanical Engineering Congress, Nov. 13-19, 2004, pp. 1-8.
- Berner, Robert A., "Tetragonal Iron Sulfide", Science, Aug. 31, 1962, vol. 137, Issue 3531, pp. 669.
- Berstein et al., "The Role of Traps in the Microstructural Control of Hydrogen Embrittlement of Steels" Hydrogen Degradation of Ferrous Alloys, Ed. T. Oriani, J. Hirth, and M. Smialowski, Noyes Publications, 1988, pp. 641-685.
- Boulegue, Jacques, "Equilibria in a sulfide rich water from Enghien-les-Bains, France", Geochimica et Cosmochimica Acta, Pergamon Press, 1977, vol. 41, pp. 1751-1758, Great Britain.
- Bruzzone et al., "Study of Hydrogen Permeation Through Passive Films on Iron Using Electrochemical Impedance Spectroscopy", PhD Thesis, 2003, Universidad Nacional del Comahue de Buenos Aires, Argentina.
- Cancio et al., "Characterization of microalloy precipitates in the austenitic range of high strength low alloy steels", Steel Research, 2002, vol. 73, pp. 340-346.
- Carboni, A., A. Pigani, G. Megahed, S. Paul, "Casting and rolling of API X 70 grades for artic application in a thin slab rolling plant", Stahl u Eisen, 2008, N° 1, p. 131-134.
- Chitwood, G. B., et al.: "High-Strength Coiled Tubing Expands Service Capabilities", as presented at the 24th Annual OTC in Houston, Texas, May 4-7, 1992, in 15 pages.
- Clark, A. Horrell, "Some Comments on the Composition and Stability Relations of Mackinawite", Neues Jahrbuch für Mineralogie, 1966, vol. 5, pp. 300-304, London, England.
- Craig, Bruce D., "Effect of Copper on the Protectiveness of Iron Sulfide Films", Corrosion, National Association of Corrosion Engineers, 1984, vol. 40, Issue 9, pp. 471-474.
- D.O.T. 178.68 Spec. 39, pp. 831-840, Non reusable (non refillable) cylinders, Oct. 1, 2002.
- Davis, J.R., et al. "ASM—Speciality Handbook—Carbon and alloy steels" ASM Speciality Handbook, Carbon and Alloy Steels, 1996, pp. 12-27, XP002364757 US.
- De Medicis, Rinaldo, "Cubic FeS, A Metastable Iron Sulfide", Science, American Association for the Advancement of Science, Steenbock Memorial Library, Dec. 11, 1970, vol. 170, Issue 3963, pp. 723-728.
- Drill Rod Joint Depth Capacity Chart, downloaded Jan. 15, 2013; <http://www.boartlongyear.com/drill-rod-joint-depth-capacity-chart>.
- Echaniz, "The effect of microstructure on the KISSL of low alloy carbon steels", NACE Corrosion '98, EE. UU., Mar. 1998, pp. 22-27, San Diego.
- Echaniz, G., Morales, C., Perez, T., "Advances in Corrosion Control and Materials in Oil and Gas Production" Papers from Eurocorr 97 and Eurocorr 98, 13, P. S. Jackman and L.M. Smith, Published for the European Federation of Corrosion, No. 26, European Federation of Corrosion Publications, 1999.
- Fang, Hong-Sheng, et al.: "The Developing Prospect of Air-cooled Bainitic Steels", International Journal of Issi, vol. 2, No. 2, Feb. 1, 2005, pp. 9-18.
- Fratin et al.: "Improving friction stir welding of blanks of different thicknesses," Materials Science and Engineering A 459 (2007).
- Gojic, Mirko and Kosec, Ladislav, , "The Susceptibility to the Hydrogen Embrittlement of Low Alloy Cr and CrMo Steels", ISIJ International, 1997, vol. 37, Issue 4, pp. 412-418.
- Gomez, G., et al.: "Air cooled bainitic steels for strong, seamless pipes—Part 1—allowy design, kinetics and microstructure", Materials Science and Technology, vol. 25, No. 12, Dec. 1, 2009. (XP002611498).
- Heckmann, et al., Development of low carbon Nb—Ti—B microalloyed steels for high strength large diameter linepipe, Ironmaking and Steelmaking, 2005, vol. 32, Issue 4, pp. 337-341.
- Hollomon, J.H., et al., Time-tempered Relations in Tempering Steel. New York Meeting, pp. 223-249, 1945.

(56)

## References Cited

## OTHER PUBLICATIONS

- Howells, et al.: "Challenges for Ultra-Deep Water Riser Systems", IIR, London, Apr. 1997, 11 pages.
- Hutchings et al., "Ratio of Specimen thickness to charging area for reliable hydrogen permeation measurement", British Corrosion Journal, 1993, vol. 28, Issue 4, pp. 309-312.
- Iino et al., "Aciers pour pipe-lines resistant au cloquage et au criquage dus a l'hydrogene", Revue de Metallurgie, 1979, vol. 76, Issue 8-9, pp. 591-609.
- Ikeda et al., "Influence of Environmental Conditions and Metallurgical Factors on Hydrogen Induced Cracking of Line Pipe Steel", Corrosion/80, National Association of Corrosion Engineers, 1980, vol. 8, pp. 8/1-8/18, Houston, Texas.
- ISO. Petroleum and natural gas industries—Materials for use in H<sub>2</sub>S-containing environments in oil and gas production. ANSI/NACE ISO, 145 pages, 2009.
- Izquierdo, et al.: "Qualification of Weldable X65 Grade Riser Sections with Upset Ends to Improve Fatigue Performance of Deepwater Steel Catenary Risers", Proceedings of the Eighteenth International Offshore and Polar Engineering Conference, Vancouver, BC, Canada, Jul. 6-11, 2008, p. 71.
- Johnston, P. W., G.Brooks, "Effect of Al<sub>2</sub>O<sub>3</sub> and TiO<sub>2</sub> Additions on the Lubrication Characteristics of Mould Fluxes", Molten Slags, Fluxes and Salts '97 Conference, 1997 pp. 845-850.
- Keizer, Joel, "Statistical Thermodynamics of Nonequilibrium Processes", Springer-Verlag, 1987.
- Kishi, T., H. Takeuegi, M.Yamamiya, H.Tsuboi, T.Nakano, T.Ando, "Mold Powder Technology for Continuous Casting of Ti-Stabilized Stainless Steels", Nippon Steel Technical Report, No. 34, Jul. 1987, pp. 11-19.
- Korolev, D. F., "The Role of Iron Sulfides in the Accumulation of Molybdenum in Sedimentary Rocks of the Reduced Zone", Geochimistry, 1958, vol. 4, pp. 452-463.
- Lee, Sung Man and Lee, Jai Young, "The Effect of the Interface Character of TiC Particles on Hydrogen Trapping in Steel", Acta Metall., 1987, vol. 35, Issue 11, pp. 2695-2700.
- Mehling, Wilfred L.: "Hot Upset Forging," ASM Handbook vol. 14, 1998, pp. 84-95.
- Mishael, et al., "Practical Applications of Hydrogen Permeation Monitoring," Corrosion, Mar. 28-Apr. 1, 2004, Corrosion 2004, Nacional Association of Corrosion Engineers, vol. Reprint No. 04476.
- Morice et al., "Möessbauer Studies of Iron Sulfides", J. Inorg. Nucl. Chem., 1969, vol. 31, pp. 3797-3802.
- Mukongo, T., P.C.Pistorius, and A.M.Garbers-Craig, "Viscosity Effect of Titanium Pickup by Mould Fluxes for Stainless Steel", Ironmaking and Steelmaking, 2004, vol. 31, No. 2, pp. 135-143.
- Mullet et al., "Surface Chemistry and Structural Properties of Mackinawite Prepared by Reaction of Sulfide Ions with Metallic Iron", Geochimica et Cosmochimica Acta, 2002, vol. 66, Issue 5, pp. 829-836.
- Murcowchick, James B. and Barnes, H.L., "Formation of a cubic FeS", American Mineralogist, 1986, vol. 71, pp. 1243-1246.
- NACE MR0175/ISO 15156-1 Petroleum and natural gas industries—Materials for use in H<sub>2</sub>S-containing Environments in oil and gas production—Part 1: General principles for selection of cracking-resistant materials, Jun. 28, 2007.
- Nagata, M., J. Speer, D. Matlock, "Titanium nitride precipitation behavior in thin slab cast high strength low alloyed steels", Metallurgical and Materials Transactions A, 2002 , vol. 33A, p. 3099-3110.
- Nakai et al., "Development of Steels Resistant to Hydrogen Induced Cracking in Wet Hydrogen Sulfide Environment", Transactions of the ISIJ, 1979, vol. 19, pp. 401-410.
- Nandan et al.: "Recent advances in friction-stir welding—Process, weldment structure and properties," Progress in Materials Science 53 (2008) 980-1023.
- Pollack, Herman, W., Materials Science and Metallurgy, Fourth Edition, pp. 96 and 97, 1988.
- Pressure Equipment Directive 97/23/EC, May 29, 1997, downloaded from website:[http://ec.europa.eu/enterprise/pressure\\_equipment/ped/index\\_en.html](http://ec.europa.eu/enterprise/pressure_equipment/ped/index_en.html) on Aug. 4, 2010.
- Prevéy, Paul, et al., "Introduction of Residual Stresses to Enhance Fatigue Performance in the Initial Design", Proceedings of Turbo Expo 2004, Jun. 14-17, 2004, pp. 1-9.
- Rickard, D.T., "The Chemistry of Iron Sulphide Formation at Low Temperatures", Stockholm Contrib. Geol., 1969, vol. 26, pp. 67-95.
- Riecke, Ernst and Bohnenkamp, Konrad, "Über den Einfluss von Gitterverstellen in Eisen auf die Wassersroffdiffusion", Z. Metallkde., 1984, vol. 75, pp. 76-81.
- Savatori et al.: European Commission Report, EUR 2006, EUR2207, 3 pp. STN\_Abstract.
- Shanabarger, M.R. and Moorhead, R. Dale, "H<sub>2</sub>O Adsorption onto clean oxygen covered iron films", Surface Science, 1996, vol. 365, pp. 614-624.
- Shoemaker, et al., "Formation of Ferrous Monosulfide Polymorphs During Corrosion of Iron by Aqueous Hydrogen Sulfide at 21 degrees C", Journal of the Electrochemical Society, 1980, vol. 127, Issue 5, pp. 1007-1015.
- Skoczylas, G., A.Dasgupta, R.Bommaraju, "Characterization of the chemical interactions during casting of High-titanium low carbon enameling steels", 1991 Steelmaking Conference Proceeding, pp. 707-717.
- Smyth, D., et al.: Steel Tubular Products, Properties and Selection: Irons, Steels, and High-Performance Alloys, vol. 1, ASM Handbook, ASM International, 1990, p. 327-336.
- Spry, Alan, "Metamorphic Textures", Pergamon Press, 1969, New York.
- Taira et al., "HIC and SSC Resistance of Line Pipes for Sour Gas Service", Nippon Kokan Technical Report, 1981, vol. 31, Issue 1-13.
- Taira et al., "Study on the Evaluation of Environmental Condition of Wet Sour Gas", Corrosion 83 (Reprint. No. 156, National Association of Corrosion Engineers), 1983, pp. 156/2-156/13, Houston, Texas.
- Takeno et al., "Metastable Cubic Iron Sulfide—With Special Reference to Mackinawite", American Mineralogist, 1970, vol. 55, pp. 1639-1649.
- Tenaris brochure. Coiled Tubes HS80CRA, 2 pages, 2008.
- Tenaris brochure. Coiled Tubes Suggested Field Welding Procedure (GTAW) for Coiled Tubing Grads HS70, HS80, HS90, HS11 0, 3 pages, 2007.
- Tenaris brochure. Coiled Tubing for Downhole Applications, 10 pages, 2007.
- Tenaris Newsletter for Pipeline Services, Apr. 2005, p. 1-8.
- Tenaris Newsletter for Pipeline Services, May 2003, p. 1-8.
- Thethi, et al.: "Alternative Construction for High Pressure High Temperature Steel Catenary Risers", OPT USA, Sep. 2003, p. 1-13.
- Thewlis, G., Weldability of X100 linepipe, Science and Technology of Welding and Joining, 2000, vol. 5, Issue 6, pp. 365-377.
- Tivelli, M., G. Cumino, A. Izquierdo, E. Anelli, A. Di Schino, "Metallurgical Aspects of Heavy Wall—High Strength Seamless Pipes for Deep Water Applications", RioPipeline 2005, Oct. 17-19, 2005, Rio (Brasil), Paper n° IBP 1008\_05.
- Todoroki, T. Ishii, K. Mizuno, A. Hongo, "Effect of crystallization behavior of mold flux on slab surface quality of a Ti-bearing Fe—Cr—Ni super alloy cast by means of continuous casting process", Materials Science and Engineering A, 2005, vol. 413-414, p. 121-128.
- Turconi, G. L.: "Improvement of resistance to SSC initiation and propagation of high strength OCTG through microstructure and precipitation control"; "Paper 01077", NACE International, Houston, TX, Mar. 16, 2001. (XP009141583).
- Vaughan, D. J. and Ridout, M.S., "Moessbauer Studies of Some Sulphide Minerals", J. Inorg. Nucl. Chem., 1971, vol. 33, pp. 741-746.
- Wegst, C.W., "Stahlüssel", Auflage 1989, Seite 119, 2 pages.
- Yu et al.: "New steels and alloys in mechanical engineering / ed.," M: Mechanical Engineering, 1976, p. 19.

\* cited by examiner

FIG. 1



FIG. 2



FIG.3

HARDNESS RATIO AND NUMBER OF TIMES  
OF MAKE-UP AND BREAK-OUT

FIG. 4A



FIG. 4B



FIG. 5A



FIG. 5B



# GALLING RESISTANT DRILL PIPE TOOL JOINT AND CORRESPONDING DRILL PIPE

## TECHNICAL FIELD

This invention relates to a drill pipe tool joint and a corresponding drill pipe, more particularly, to a drill pipe tool joint and a corresponding drill pipe, which has optimized surface hardness for repeating make-up/break-out operation without the use of a screw grease when drill pipes used in well drilling for oil, natural gas, shale gas, geothermal and the like are screwed together, thereby being environment-friendly, as well as improving operating efficiency.

## BACKGROUND ART

Drill pipes used in drilling wells for oil, natural gas, and the like have been connected by tool joints. In order for the tool joints to transmit high torque required during drilling, an outer diameter portion thereof is formed to be greater than an outer diameter of a pipe body, while an inner diameter portion thereof is formed to be smaller than an inner diameter of the pipe body. To this end, generally, a make-up torque value during joining a pin and a box of the tool joints is required to be several times a make-up torque value for casing or tubing used in wells for production of oil, natural gas, and the like.

On the other hand, for the number of times of make-up/break-out operations of the pin and the box of the threaded joints for the casing or tubing used in wells for production, the number of tripings is not so many. Therefore, for anti-galling (scoring) evaluation testing, International Organization for Standardization standard ISO13679 defines acceptance/rejection determination in performance evaluation for 2 times of make-up/break-out operation in the casing and for 9 times of make-up/break-out operation in the tubing. However, the drill pipes require drill bit replacement according to drilling conditions of each type such as geological strata, well inclination, depth, and the like. Further, there is no ISO standard definition for the drill pipes, but the galling resistance is expected to be not less than 25 trips, and more preferably not less than 50 trips.

For the casing or tubing, a lubricating grease (or dope) to be applied to the pin and the box of the threaded joints has been used for anti-galling, and also a surface treatment such as plating has been employed (see here bellow patent literatures 1 to 7). However, spreading due to tool joint cleaning, excess lubricating grease deposition on well bottom due to coating, rig pollution emission in workplace, etc. may have adverse effects on the environment. Therefore, for environmental consideration, alternative surface coating treatment using no conventional screw lubricating grease, so-called "grease-free" or "dope-free", i.e., with no lubricating grease (nor dope) to be applied to the pin and the box of the threaded joints, has recently been put into practical use.

Following documents have been identified that relate to the said technical field:

## PATENT LITERATURE CITATION LIST

- Patent Literature 1: WO2003-060198
- Patent Literature 2: WO2005-098300
- Patent Literature 3: WO2007-026970
- Patent Literature 4: WO2008-108263
- Patent Literature 5: JP-A-2003-074763

Patent Literature 6: U.S. Pat. No. 4,758,025  
Patent Literature 7: U.S. Pat. No. 4,468,309

Patent Literature 1 discloses a tubular member in which at least one of a pin and a box is coated with an alloy of copper and tin which contains 20 wt % to 80 wt % copper.

Patent Literature 2 discloses a threaded joint for steel pipes in which at least one of a pin and a box is furnished with a solid lubricant coating comprising a binder, copper powder and lubricating powder at its surface and the other of the pin and the box is coated with zinc or zinc alloy coating.

Patent Literature 3 discloses a threaded joint for steel pipes in which Sn—Bi alloy plating or Sn—Bi—Cu alloy plating is formed on at least one of a pin and a box.

Patent Literature 4 discloses a screw joint for steel pipe in which at least one of a pin and a box is covered with a first plating layer of Cu—Zn alloy or Cu—Zn-M1 alloy (M1 is at least one selected from among Sn, Bi and In), and a second plating layer of Sn-M2 alloy (M2 is at least one element selected from among Bi, In, Ni, Zn and Cu).

Patent Literature 5 discloses a joint for an oil well pipe in which a first plating layer comprising the first to the nth layers of Cu—Sn alloy plating is formed on a box.

Patent Literature 6 discloses a method for preventing galling comprising providing a soft metal coating such as an electroless metal conversion coating of Cu or Zn on at least one of a pin and a box, and coating a lubricant agent thereon.

Patent Literature 7 discloses a method for resisting galling including depositing a material film having a low shear stress value such as gold, silver, lead, tin, indium, palladium or copper by ion plating on at least one of a pin and a box.

Although Patent Literatures 1 to 7 disclose examples of solid lubricant, a technique for achieving repetitive make-up/break-out operations of a drill pipe tool joint for not less than 25 times without any use of a lubricating grease has not been found.

## SUMMARY OF INVENTION

### Technical Problem

However, as it stands, there exists no substitutable surface coating treatment using no screw lubricating grease for the drill pipe tool joints.

There is furthermore a constant need of improving galling resistance and achieving an increasing number of repetitive make-up/break-out operations of a drill pipe tool joint.

Accordingly, it is an object of the present invention to provide a drill pipe tool joint and a corresponding drill pipe, which can be subject to repetitive make-up/break-out operations for not less than 25 times without any use of a lubricating grease for avoiding galling, which is environment-friendly, and which does not use a lubricant.

### Solution to Problem

The said technical problem is solved thanks to a drill pipe tool joint comprising: a pin including a male threaded portion at an outer surface; and

60 a box including a female threaded portion at an inner surface, the female threaded portion to be screwed and fastened to the male threaded portion in a contacting zone consisting of a male threaded contacting surface and a female threaded contacting surface, wherein at least a portion of the male threaded contacting surface or a portion of the female threaded contacting surface is a surface layer consisting of a hard metal and respectively at least a portion of the female threaded

contacting surface or a portion of the male threaded contacting surface is a surface layer consisting of a soft material and where said both surface portions are contacting surfaces after screwing.

The present invention is also directed to a drill pipe comprising:

a pipe body; and

a pin including a male threaded portion at an outer surface; and

a box including a female threaded portion at an inner surface, the female threaded portion to be screwed and fastened to a male threaded portion of another drill pipe of the same kind, in a contacting zone consisting of a male threaded contacting surface and a female threaded contacting surface;

wherein at least a portion of the male threaded contacting surface or a portion of the female threaded contacting surface is a surface layer consisting of a hard metal and respectively at least a portion of the female threaded contacting surface or a portion of the male threaded contacting surface is a surface layer consisting of a soft material and where said both surface portions are contacting surfaces after screwing.

A plurality of said drill pipes will comprise, after being assembled, a plurality of preceding drill pipe tool joints.

Therefore the said drill pipe tool joint and drill pipe relate to a group of inventions so linked as to form a single general inventive concept.

The drill pipe tool joint or the drill pipe according to the present invention may also comprise following features that may be combined according to all possible embodiments:

the surface layers consisting respectively of a hard metal and of a soft material occupy at least 90% of the contacting zone surfaces;

the male threaded contacting surface or the female threaded contacting surface is a surface layer consisting of a hard metal and respectively the female threaded contacting surface or the male threaded contacting surface is a surface layer consisting of a soft material; the hardness of the hard metal is equal or greater than 600 Hv, for example equal or greater than 800 Hv;

the hardness of the soft material is equal or lower than

350 Hv, for example equal or greater than 150 Hv; the hardness ratio of the hard metal to the soft material

is equal or greater than 2.8, for example equal or greater than 5;

the hard metal substantially consists of a metal chosen within the list consisting of chromium (Cr), nickel (Ni), or their mixture; according to an embodiment, said layer of hard metal is obtained through a plating process; according to an embodiment, the layer of hard metal is made of hard chromium plating; according to another embodiment, the layer of hard metal is made non electric nickel plating;

the thickness of the layer of hard metal is comprised between 5 to 100  $\mu\text{m}$ , for example equal or greater than 10  $\mu\text{m}$ , for example equal or less than 50  $\mu\text{m}$ ;

the soft material consists of a metal chosen within the list consisting of copper (Cu), zinc, (Zn), or their mixture; according to an embodiment, said layer of soft material is obtained through a plating process; according to an embodiment, the layer of soft material is made of electrolytic copper or of electrolytic zinc;

the soft material substantially consists of a phosphate layer;

the thickness of the layer of soft material is comprised between 5 to 100  $\mu\text{m}$ , for example equal or greater than 10  $\mu\text{m}$ , for example equal or less than 50  $\mu\text{m}$ ; the drill pipe tool joint is devoid of dope or of lubricant grease;

the pin including the male threaded portion and the box including the female threaded portion are devoid of dope or of lubricant grease when being screwed and fastened for assembling.

According to the present invention the hardness of a layer is determined as Vickers hardness (Hv).

According to the present invention, one has to understand the wordings "hard" and "soft" as relative wordings; a surface layer consisting of a soft material has thus hardness lower than a surface layer consisting of a hard material.

The present invention also relates to a method of assembling preceding drill pipes wherein the pins including the male threaded portion and the boxes including the female threaded portion are devoid of dope or of lubricant grease when being screwed and fastened for assembling.

#### Advantageous Effects of Invention

According to the invention, it is possible to provide a drill pipe tool joint and a corresponding drill pipe, which can be subject to repetitive make-up/break-out operations for not less than 25 times without any use of lubricating grease for suppressing galling, which is environment-friendly, and which does not use a lubricant.

#### BRIEF DESCRIPTION OF DRAWINGS

FIG. 1 is a diagram showing a whole structure of a drill pipe tool joint and a drill pipe with that drill pipe tool joint in an embodiment according to the invention.

FIG. 2 is a longitudinal cross-sectional view showing the drill pipe in the embodiment according to the invention.

FIG. 3 is a graph showing the relationship between the hardness ratio of the hard metal to the soft material and the number of times of make-up/break-out operation of the drill pipe tool joint in the embodiment according to the invention.

FIG. 4A is a photograph showing a surface state of a pin after make-up/break-out testing for the drill pipe tool joint in the embodiment according to the invention.

FIG. 4B is a photograph showing a surface state of a box after the make-up/break-out testing for the drill pipe tool joint in the embodiment according to the invention.

FIG. 5A is a photograph showing a surface state of a pin on which the galling occurred after make-up/break-out testing for a drill pipe tool joint.

FIG. 5B is a photograph showing a surface state of a box on which the galling occurred after the make-up/break-out testing for the drill pipe tool joint.

#### DESCRIPTION OF EMBODIMENTS

##### Structure of Drill Pipe Tool Joint

FIG. 1 is a diagram showing a whole structure of a drill pipe tool joint and a drill pipe with that drill pipe tool joint, in an embodiment according to the invention. In addition, FIG. 2 is a longitudinal cross-sectional view showing the drill pipe in the embodiment according to the invention. The drill pipe tool joint for drilling is defined by the API (American Petroleum Institute) standard, and is formed in several shapes with different details, such as a shape as shown in FIGS. 1 and 2.

A drill pipe tool joint 1 in an embodiment according to the invention comprises a pin 2 including a male threaded portion 23 at an outer surface 21, a box 3 including a female threaded portion 33 at an inner surface 31. The female threaded portion 33 is to be screwed and fastened to the male threaded portion 23 in a contacting zone consisting of a male threaded contacting surface and a female threaded contacting surface. At least a portion of the male threaded contacting surface or a portion of the female threaded contacting surface is a surface layer consisting of a hard metal and respectively at least a portion of the female threaded contacting surface or a portion of the male threaded contacting surface is a surface layer consisting of a soft material and said both surface portions are contacting surfaces after screwing.

Namely, the screwed surface (21 or 31) of the one of the male threaded portion 23 and the female threaded portion 33 includes a surface layer consisting of a hard metal, while the screwed surface (31 or 21) of the other thereof includes a surface layer consisting of a soft material which is lower in hardness than the surface layer consisting of a hard metal.

More concretely, the screwed surface (21 or 31) of the one of the male threaded portion 23 and the female threaded portion 33 has a layer or structure having a first hardness as an outermost surface entirely around the screwed surface thereof, while the screwed surface (31 or 21) of the other thereof has a layer or structure having a second hardness as an outermost surface entirely around the screwed surface thereof, in which the second hardness is lower in hardness than the first hardness.

A drill pipe 4 in another embodiment according to the invention comprises a pipe body 50, a pin 2 including a male threaded portion 23 at an outer surface 21 and a box 3 including a female threaded portion 33 at an inner surface 31. The female threaded portion is to be screwed and fastened to a male threaded portion of another drill pipe of the same kind, in a contacting zone consisting of a male threaded contacting surface and a female threaded contacting surface. At least a portion of the male threaded contacting surface or a portion of the female threaded contacting surface is a surface layer consisting of a hard metal and respectively at least a portion of the female threaded contacting surface or a portion of the male threaded contacting surface is a surface layer consisting of a soft material and said both surface portions are contacting surfaces after screwing.

The drill pipe 4 is used in drilling by fastening (referred to as "make-up") and connecting a plurality of drill pipes 4 with the drill pipe tool joints 1. Here, the drill pipe tool joint 1 comprises the male threaded portion 23 provided at the outer surface 21 of the pin 2 of the drill pipe 4, and the female threaded portion 33 provided at the inner surface 31 of the box 3 of the other drill pipe 4. The male threaded portion 23 provided at the outer surface 21 of the pin 2 of the drill pipe 4 and the female threaded portion 33 provided at the inner surface 31 of the box 3 of the other drill pipe 4 are screwed and fastened together. In addition, the drill pipes 4 are unfastened (referred to as "break-out") as necessity. Therefore, the drill pipes 4 are subject to repetitive make-up/break-out operations at the drill pipe tool joint 1.

The male threaded portion 23 formed at the outer surface 21 of the pin 2 includes the surface layer consisting of a hard metal having the first hardness (i.e. hard surface-treated surface), or the surface layer consisting of a soft material having the second hardness provided by a surface layer

consisting of a soft material (i.e. soft surface-treated surface), in which the second hardness is lower in hardness than the first hardness.

As examples of the hard metal, there are listed chromium plating, hard chromium plating, nickel plating, non-electric nickel plating, etc.

Also, as examples of the surface layer consisting of a soft material at the lower hardness than the hard metal surface treatment described above, there are listed a copper plating, 10 electrolytic copper plating, zinc plating, electrolytic zinc plating, etc. Further, surface layer consisting of a soft material is not limited to the plating, but a phosphating such as manganese phosphating and zinc phosphating may be employed, namely a phosphate layer may be formed.

15 According to embodiments of the present invention, the hardness of the hard metal is equal or greater than 600 Hv, for example equal or greater than 800 Hv.

According to embodiments of the present invention, the hardness of the soft material is equal or lower than 350 Hv, 20 for example equal or greater than 150 Hv.

According to embodiments of the present invention, the thickness of the layer of hard metal is comprised between 5 to 100  $\mu\text{m}$ , for example equal or greater than 10  $\mu\text{m}$ , for example equal or less than 50  $\mu\text{m}$ .

25 According to embodiments of the present invention, the thickness of the layer of soft material is comprised between 5 to 100  $\mu\text{m}$ , for example equal or greater than 10  $\mu\text{m}$ , for example equal or less than 50  $\mu\text{m}$ .

On the other hand, the female threaded portion 33 formed 30 at the inner surface 31 of the box 3 has a surface-treated surface which is surface-treated differently from the surface-treated surface of the male threaded portion 23. More concretely, the female threaded portion 33 has a layer or a structure (including metal structure) having the second hardness at its outermost surface. When the male threaded portion 23 has the surface-treated surface having the first hardness, the female threaded portion 33 has the surface-treated surface having the second hardness, which is lower in hardness than the first hardness (i.e. soft surface-treated surface). Alternatively, when the male threaded portion 23 35 has the surface-treated surface having the second hardness, the female threaded portion 33 has the surface-treated surface having the first hardness.

The drill pipes 4 with the male threaded portion 23 and the 40 female threaded portion 33 configured as described above are fastened together with the drill pipe tool joint 1. In other words, the drill pipes 4 are fastened together by screwing the male threaded portion 23 to the female threaded portion 33.

The male threaded portion 23 has a surface layer consisting of a soft material or a surface layer consisting of a hard metal as described above, and the female threaded portion 33 has a surface layer consisting of a hard metal or a surface layer consisting of a soft material described above. More concretely, when the male threaded portion 23 has a surface 50 layer consisting of a hard metal, the female threaded portion 33 has a surface layer consisting of a soft material. Alternatively, when the male threaded portion 23 has a surface layer consisting of a soft material, the female threaded portion 33 has a surface layer consisting of a hard metal.

55 In the drill pipe tool joint 1, the male threaded contacting surface or the female threaded contacting surface is a surface layer consisting of a hard metal and respectively the female threaded contacting surface or the male threaded contacting surface is a surface layer consisting of a soft material.

60 Other embodiments within the scope of the present invention may have contacting zone surfaces with surface layers consisting of a hard metal and/or of a soft material occupy-

ing only partially the contacting zone surfaces; according to an embodiment, the surface layers consisting respectively of a hard metal and of a soft material occupy at least 90% of the contacting zone surfaces.

In the drill pipe tool joint 1 thus configured, even though the make-up/break-out operation is repeatedly performed between the female threaded portion 33 and the male threaded portion 23, the occurrence of so-called "galling" is suppressed. Therefore, the number of times of make-up/break-out operation until the occurrence of galling can be increased.

Here, the "galling" represents the state of the damage caused by the contact between the metals. The "advance to galling from seizure (welding)" refers to a state that a contact surface is seized and does not move at the initial seizure then further rotated or moved so that the seized surface exfoliates and is damaged. This galling is likely to occur in the case that a contact surface pressure is high or that an affinity between rubbing metals is high.

In the present embodiment, the male threaded portion 23 and the female threaded portion 33 have the surface layer consisting of a hard metal and the surface layer consisting of a soft material that are different in hardness from each other, respectively, so that the affinity between surfaces to be in contact with each other is low. Further, it is preferable to set a hardness ratio of the hard metal to the soft material to be not less than 2.8 as described later. According to an embodiment said hardness ratio of the hard metal to the soft material equal or greater than 5. According to this structure, it is possible to suppress the occurrence of galling, thereby increase the number of times of make-up/break-out operations until the occurrence of galling. It should be noted that the number of times of make-up/break-out operations of the drill pipe tool joint 1 is demanded strictly compared with those of conventional threaded tool joint for a casing and

tubing for wells for production, so that the number of times of make-up/break-out operations is preferably not less than 25 times, more preferably not less than 50 times.

## EXAMPLES

### Make-Up/Break-Out Testing

In order to carry out an anti-galling evaluation in make-up/break-out operation of the drill pipe tool joint 1, a make-up/break-out testing was conducted by using a drill pipe with a size of 5½ FH. The drill pipe of 5½ FH has an outer diameter of 7 inches (177.8 mm) and an inner diameter of 3.75 inch (95.25 mm). Material grade is TJ130 (AISI modified 4135. Yield strength 130-150 ksi, Tensile strength Min. 140 ksi). Surface treatment area is from corner of the external shoulder through threads to the internal shoulder or internal bevel. After repeating make-up/break-out operations of the drill pipe, the number of times of make-up/break-out operations until the galling occurs at a surface of the male threaded portion 23 or the female threaded portion 33 was evaluated. The evaluation result is preferably not less than 25 times, more preferably not less than 50 times.

Table 1 shows the results of the make-up/break-out testing. The combinations of the surface treatments provided on the surfaces of the male threaded portion 23 and the female threaded portion 33 are as follows: the pin is coated with copper plating, chromium plating, or nickel plating, and the box is provided with copper plating, zinc plating, manganese phosphating, or no surface treatment (i.e. as machined without any surface treatment, which is indicated as "none" in the item of "surface treatment"). The number of times of make-up/break-out operations until the occurrence of galling is evaluated for each of these samples. For the plating thickness, a range of not less than 10 µm and less than 30 µm, which is available for industrial purpose, was selected.

TABLE I

|                       | Pin               |                | Box                   |                | Hardness Ratio | The number of times of make-up/break-out until the occurrence of galling |
|-----------------------|-------------------|----------------|-----------------------|----------------|----------------|--------------------------------------------------------------------------|
|                       | Surface Treatment | Thickness (µm) | Surface Treatment     | Thickness (µm) |                |                                                                          |
| Example 1             | Cr plating        | 10-20          | Cu plating            | 20-30          | 6.37           | No occurrence of galling even after 100 times of repetitions             |
| Example 2             | Ni plating        | 10-20          | Cu plating            | 20-30          | 6.64           | No occurrence of galling even after 100 times of repetitions             |
| Example 3             | Cr plating        | 10-20          | Cu plating            | 10-20          | 6.37           | 74 times                                                                 |
| Example 4             | Ni plating        | 10-20          | Cu plating            | 10-20          | 6.64           | 69 times                                                                 |
| Example 5             | Cr plating        | 10-20          | Zn plating            | 10-20          | 9.24           | 64 times                                                                 |
| Example 6             | Ni plating        | 10-20          | Zn plating            | 10-20          | 9.64           | 58 times                                                                 |
| Example 7             | Cr plating        | 10-20          | Manganese phosphating | 10-20          | 2.80           | 25 times                                                                 |
| Example 8             | Cr plating        | 10-20          | Manganese phosphating | 10-20          | 2.80           | 26 times                                                                 |
| Example 9             | Ni plating        | 10-20          | Manganese phosphating | 10-20          | 2.92           | 25 times                                                                 |
| Comparative Example 1 | Cu plating        | 10-20          | Cu plating            | 10-20          | 1.00           | 1 time                                                                   |
| Comparative Example 2 | Cu plating        | 10-20          | Cu plating            | 20-30          | 1.00           | 13 times                                                                 |

TABLE I-continued

|                       | Pin               |                | Box                   |                | Hardness Ratio | The number of times of make-up/break-out until the occurrence of galling |
|-----------------------|-------------------|----------------|-----------------------|----------------|----------------|--------------------------------------------------------------------------|
|                       | Surface Treatment | Thickness (μm) | Surface Treatment     | Thickness (μm) |                |                                                                          |
| Comparative Example 3 | Cu plating        | 10-20          | Manganese phosphating | 10-20          | 2.27           | 1 time                                                                   |
| Comparative Example 4 | Cu plating        | 10-20          | None                  | 10-20          | 2.50           | 1 time                                                                   |
| Comparative Example 5 | Cu plating        | 20-30          | Cu plating            | 10-20          | 1.00           | 15 times                                                                 |
| Comparative Example 6 | Cu plating        | 20-30          | Manganese phosphating | 10-20          | 2.27           | 6 times                                                                  |
| Comparative Example 7 | Cu plating        | 20-30          | None                  | —              | 2.50           | 1 time                                                                   |
| Comparative Example 8 | Cu plating        | 10-20          | None                  | —              | 2.50           | 1 time                                                                   |

From the results of Table 1, it was found that in the cases that the pin 2 and the box 3 are provided with a surface layer consisting of a hard metal and a surface layer consisting of a soft material that are different from each other, the make-up/break-out operations without any occurrence of galling can be conducted for not less than 25 times, so that the galling resistance is good (in Examples 1 to 9). Particularly, in the cases that the chromium plating or nickel plating is applied to the pin 2 while the copper plating or zinc plating is applied to the box 3, the make-up/break-out operations without any occurrence of galling can be conducted for not less than 50 times (in Examples 1 to 6). The combination of the surface layer consisting of a hard metal and the surface layer consisting of a soft material, more concretely, the combinations of the chromium plating or nickel plating and the copper plating or zinc plating have the interchangeability so that they may be applied on either side to of the box 3 and the pin 2. In Table 1, "Cr plating" is hard Cr plating, "Ni plating" is electroless Ni—P plating, "Cu plating" is electrolytic Cu plating, and "Zn plating" is electrolytic Zn plating.

#### Hardness Measurement

From the results of the make-up/break-out testing described above, it was found that the galling resistance would be excellent when the pin 2 and the box 3 are provided with the hard surface treatment and soft surface treatment that are different from each other in hardness. Then, the hardness of each of the hard surface treatment and the soft surface treatment was studied as parameter.

Table 2 shows the measurement results of the surface hardness of the surface treatment provided for each of the pin 2 and the box 3, in which the hardness in each of Nos. 1 to 6 according to the type of the surface treatment is shown by Vickers hardness (Hv). The Vickers hardness test method was performed in accordance with ISO 6507-1 and ISO 6507-4. The measurement was carried out for plural times, and an average value thereof is shown as the hardness (average Hv). Further, in the case of plating, the hardness of the plating material itself can be used instead of the measured value as the hardness of each surface treatment. As described above, the type of the surface treatment corresponds to the type of the surface treatment in Examples 1 to 9 and comparative examples 1 to 8 in Table 1.

TABLE 2

| Type of surface treatment                    | Hardness (average Hv) |
|----------------------------------------------|-----------------------|
| 1 Non electric Ni P plating                  | 877                   |
| 2 Hard Cr plating                            | 841                   |
| 3 Electrolytic Cu plating                    | 132                   |
| 4 Electrolytic Zn plating                    | 91                    |
| 5 Manganese phosphating                      | 300                   |
| 6 Drill pipe tool joint material as machined | 330                   |

The relationship between the hardness ratio of the hard metal to the soft material and the number of times of make-up/break-out operations is now discussed.

FIG. 3 is a graph showing the relationship between the hardness ratio of the hard metal to the soft material and the number of times of make-up/break-out from the results in Table 1 and Table 2. According to FIG. 3, when the hardness ratio of the hard metal to the soft material is not less than 2.8, the number of times of make-up/break-out operations without any occurrence of galling is increased to be not less than 25 times. Results are furthermore increased when the hardness ratio of the hard metal to the soft material is equal or greater to 5, as for an example equal or greater than 6.

FIG. 4A is a photograph showing a surface state of a pin after make-up/break-out testing for the drill pipe tool joint in the embodiment according to the invention, and FIG. 4B is a photograph showing a surface state of a box after the make-up/break-out testing for the drill pipe tool joint in the embodiment according to the invention. FIG. 5A is a photograph showing a surface state of a pin on which the galling occurred after make-up/break-out testing for a drill pipe tool joint, and FIG. 5B is a photograph showing a surface state of a box on which the galling occurred after the make-up/break-out testing for the drill pipe tool joint.

In the make-up/break-out testing as shown in Table 1, no galling occurred at the chromium plated surface of the pin 2 and the copper plated surface of the box 3 even after repeating the make-up/break-out operation for not less than 50 times as shown in FIGS. 4A and 4B.

On the contrary, in the make-up/break-out testing as shown in Table 1, galling occurred at a conventionally-used copper plated surface (plating thickness of 10-20 μm) of the pin 2 and the heavier copper plated surface (plating thickness of 20-30 μm) of the box 3 after repeating the make-up/break-out operation for around 10 times as shown in FIGS. 5A and 5B.

## 11

Advantages of the embodiment of the present invention are further exemplified.

According to the drill pipe tool joint and the corresponding drill pipe in the embodiment of the present invention, following advantages can be achieved.

(1) In the present embodiment, the male threaded portion 23 and the female threaded portion 33 have the surface layer consisting of a hard metal and the surface layer consisting of a soft material that are different in hardness from each other, respectively. Since the male threaded portion 23 and the female threaded portion 33 have the surface-treated surfaces having the different hardness, e.g., the combination of chromium plating and copper plating, respectively, the affinity between screwed surfaces in contact with each other is low. Thus, even though the make-up/break-out operation is performed repeatedly between the male threaded portion 23 and the female threaded portion 33, the occurrence of so-called "galling" can be suppressed. Therefore, the number of times of make-up/break-out operations until the occurrence of galling can be increased.

(2) From the relationship between the hardness ratio of the hard metal to the soft material and the number of times of make-up/break-out operations as shown in FIG. 3, it is confirmed that when the hardness ratio of the hard metal to the soft material is not less than 2.8, the number of times of make-up/break-out operations without any occurrence of galling is increased, particularly, the make-up/break-out operations for not less than 25 times as a practicable range for the drill pipe tool joint is possible. In the case that chromium plating or nickel plating is applied to the pin 2 while copper plating is applied to the box 3, the make-up/break-out operations until the occurrence of galling for not less than 50 times can be achieved.

(3) By applying the combination of the surface treatment with different hardness such as the combination of chromium plating and copper plating to the pin 2 and the box 3, the conventionally-used lubricating grease (or dope) is no longer required to be applied to the pin 2 and the box 3. Therefore, it is possible to achieve an environment-friendly drill pipe tool joint and a drill pipe with the same.

(4) By applying the combination of surface-treated surfaces having the hardness ratio of the hard metal to the soft material of not less than 2.8 to the screwed surfaces of the pin 2 and the box 3 that are subject to repetitive make-up/break-out operations, it is possible to achieve a significant advantage that the number of times of make-up/break-out operations without any occurrence of galling increases. From the graph of FIG. 3, it is understood that the hardness ratio of the hard metal to the soft material of 2.8 has a criticality, since the number of times of make-up/break-out operations without any occurrence of galling significantly changes before and after the hardness ratio of the hard metal to the soft material of 2.8. As shown by FIG. 3, results are furthermore increased when the hardness ratio of the hard metal to the soft material is equal or greater to 5, as for an example equal or greater than 6.

Although the invention has been described with respect to the specific embodiments, these embodiments are merely examples and do not limit the invention according to claims. These novel embodiments and modifications can be enforced in other various manners, and various omissions, replacements, alterations and the like may be made without

## 12

going beyond the gist of the invention. All the combinations of the features described in the embodiments are not necessarily essential for the means for solving the problem of the Invention. Further, these embodiments and modifications are included in the scope and gist of the invention and the scope of the inventions described in claims and their equivalents.

## INDUSTRIAL APPLICABILITY

A drill pipe tool joint and a corresponding drill pipe according to the present invention can be used without the use of a screw grease when the make-up/break-out operations of the drill pipe are performed for not less than 25 times, thereby being environment-friendly, as well as improving operating efficiency.

## REFERENCE SIGNS LIST

- 1 Drill pipe tool joint
- 2 Pin
- 3 Box
- 4 Drill pipe
- 21 Outer surface of Pin
- 23 Male threaded portion
- 31 Inner surface of Box
- 33 Female threaded portion
- 50 Pipe body

The invention claimed is:

1. A dope-free drill pipe tool joint comprising:  
a pin including a male threaded portion at an outer surface; and  
a box including a female threaded portion at an inner surface, the female threaded portion to be screwed and fastened to the male threaded portion in a contacting zone consisting of a male threaded contacting surface and a female threaded contacting surface;  
wherein at least a portion of the male threaded contacting surface or a portion of the female threaded contacting surface is a surface layer consisting of a hard metal and respectively at least a portion of the female threaded contacting surface or a portion of the male threaded contacting surface is a surface layer consisting of a soft material and where said both surface portions are contacting surfaces after screwing;  
wherein the drill pipe tool joint is dope free;  
wherein a hardness ratio of the hard metal to the soft material is equal or greater than 2.8; and  
wherein the hardness ratio allows the pin and the box to be made up and broken out at least 25 times without any occurrence of galling.

2. The drill pipe tool joint of claim 1, wherein the male threaded contacting surface or the female threaded contacting surface is a surface layer consisting of a hard metal and respectively the female threaded contacting surface or the male threaded contacting surface is a surface layer consisting of a soft material.

3. The drill pipe tool joint of claim 1, wherein the hardness of the hard metal is equal or greater than 600 Hv.

4. The drill pipe tool joint of claim 1, wherein the hardness of the soft material is equal or lower than 350 Hv.

5. The drill pipe tool joint of claim 1, wherein the hard metal substantially consists of a metal chosen within the list consisting of chromium (Cr), nickel (Ni), or their mixture.

6. The drill pipe tool joint of claim 5, wherein the layer of hard metal is obtained through a plating process.

## 13

7. The drill pipe tool joint of claim 1 wherein the thickness of the layer of hard metal is comprised between 5 to 100  $\mu\text{m}$ .

8. The drill pipe tool joint of claim 1, wherein the layer of soft material is obtained through a plating process.

9. The drill pipe tool joint of claim 1 wherein the thickness of the layer of soft material is comprised between 5 to 100  $\mu\text{m}$ .

10. A method of assembling the drill pipe tool joint of claim 1, wherein the pin including the male threaded portion and the box including the female threaded portion are devoid of dope or of lubricant grease during make-up.

11. The drill pipe tool joint of claim 1, wherein the hardness ratio is between 2.8 and 10.

12. The drill pipe tool joint of claim 1, wherein the hardness ratio allows the pin and the box to be made up and broken out at least 50 times without any occurrence of galling.

13. The drill pipe tool joint of claim 1, wherein the soft material consists of a metal chosen within the list consisting of copper (Cu), zinc (Zn), or their mixture.

14. The drill pipe tool joint of claim 1, wherein the soft material substantially consists of a phosphate layer.

15. A dope-free drill pipe comprising:

a pipe body; and

a pin including a male threaded portion at an outer surface; and

a box including a female threaded portion at an inner surface, the female threaded portion to be screwed and fastened to a male threaded portion of another drill pipe of the same kind, in a contacting zone consisting of a male threaded contacting surface and a female threaded contacting surface;

wherein at least a portion of the male threaded contacting surface or a portion of the female threaded contacting surface is a surface layer consisting of a hard metal and respectively at least a portion of the female threaded contacting surface or a portion of the male threaded contacting surface is a surface layer consisting of a soft material and where said both surface portions are contacting surfaces after screwing;

wherein the drill pipe is dope free;

wherein a hardness ratio of the hard metal to the soft material is equal or greater than 2.8; and

wherein the hardness ratio allows the pin and the box to be made up and broken out at least 25 times without any occurrence of galling.

16. The drill pipe of claim 15, wherein the male threaded contacting surface or the female threaded contacting surface is a surface layer consisting of a hard metal and respectively the female threaded contacting surface or the male threaded contacting surface is a surface layer consisting of a soft material.

17. The drill pipe of claim 15, wherein the hardness of the hard metal is equal or greater than 600 Hv.

18. The drill pipe of claim 15, wherein the hardness of the soft material is equal or lower than 350 Hv.

19. The drill pipe of claim 15, wherein the hard metal substantially consists of a metal chosen within the list consisting of chromium (Cr), nickel (Ni), or their mixture.

20. The drill pipe of claim 19, wherein the layer of hard metal is obtained through a plating process.

## 14

21. The drill pipe of claim 15, wherein the thickness of the layer of hard metal is comprised between 5 to 100  $\mu\text{m}$ .

22. The drill pipe of claim 15, wherein the layer of soft material is obtained through a plating process.

23. The drill pipe of claim 15, wherein the thickness of the layer of soft material is comprised between 5 to 100  $\mu\text{m}$ .

24. A method of assembling the drill pipe of claim 15, wherein the pin including the male threaded portion and the box including the female threaded portion are devoid of dope or of lubricant grease during make-up.

25. The drill pipe of claim 15, wherein the hardness ratio is between 2.8 and 10.

26. The drill pipe of claim 15, wherein the hardness ratio allows the pin and the box to be made up and broken out at least 50 times without any occurrence of galling.

27. The drill pipe of claim 15, wherein the soft material consists of a metal chosen within the list consisting of copper (Cu), zinc (Zn), or their mixture.

28. The drill pipe of claim 15, wherein the soft material substantially consists of a phosphate layer.

29. A dope-free drill pipe tool joint comprising:

a pin including a male threaded portion at an outer surface; and

a box including a female threaded portion at an inner surface, the female threaded portion configured to be screwed and fastened to the male threaded portion in a contacting zone consisting of a male threaded contacting surface and a female threaded contacting surface; wherein at least a portion of the male threaded contacting surface or a portion of the female threaded contacting surface is a surface layer consisting of a hard metal and respectively at least a portion of the female threaded contacting surface or a portion of the male threaded contacting surface is a surface layer consisting of a soft material and where said both surface portions are contacting surfaces after screwing;

wherein the drill pipe tool joint is dope free; and

wherein a hardness ratio of the hard metal to the soft material is between 2.8 and 10.

30. A dope-free drill pipe comprising:

a pipe body; and

a pin including a male threaded portion at an outer surface; and

a box including a female threaded portion at an inner surface, the female threaded portion to be screwed and fastened to a male threaded portion of another drill pipe of the same kind, in a contacting zone consisting of a male threaded contacting surface and a female threaded contacting surface;

wherein at least a portion of the male threaded contacting surface or a portion of the female threaded contacting surface is a surface layer consisting of a hard metal and respectively at least a portion of the female threaded contacting surface or a portion of the male threaded contacting surface is a surface layer consisting of a soft material and where said both surface portions are contacting surfaces after screwing;

wherein the drill pipe is dope free; and

wherein a hardness ratio of the hard metal to the soft material is between 2.8 and 10.

\* \* \* \* \*